

## UNITED STATES PATENT OFFICE

2,641,559

METHOD OF CLEANING AND DESCALING  
FERROUS ARTICLES AND A BATH THEREFOR

Matti H. Pakkala and Freeman J. Phillips, Pittsburgh, Pa., assignors to United States Steel Corporation, a corporation of New Jersey

No Drawing. Application September 8, 1948,  
Serial No. 48,328

6 Claims. (Cl. 134—3)

1

This invention relates to the cleaning of ferrous articles and to a bath therefor, and more particularly to the removal of scale or oxide from the surfaces of such articles. The invention may be used to clean ferrous articles in general, but is of particular advantage in the cleaning and descaling of articles of chromium or chromium-nickel steels known as stainless, corrosion-resistant and heat-resistant steels.

In general, these steels contain more than 4% chromium and are made in electric furnaces, their fabrication involving casting into ingots and subsequent conventional hot working, heat treating, and, usually, cold-working operations, to produce the desired articles. During the hot-working and heat-treating operations the surfaces of all such steels become oxidized from exposure to furnace gases or air while at the elevated temperatures to which they are heated. In addition, the surfaces may gather other matter such as spots of oil or grease.

Because of their compositions, the oxidation products formed on the surfaces of these steels during the various hot-working and heat-treating operations adhere tightly to the surfaces and are generally as resistant to chemical attack as the steels themselves. The processes used heretofore to remove these surface oxidation products may be classified as mechanical and chemical, the former including such operations as sand or shot blasting, grinding and milling, and the latter including such processes as pickling, that is, treatment in hot solutions of acid, and treatment in fused baths.

Mechanical cleaning of such steels by sand or shot blasting is expensive and has the further objection that the surfaces are roughened and to some extent hardened, as in cold working. As a consequence, such mechanical cleaning methods for such metals have been practically abandoned.

Pickling also has been found to be unsatisfactory since it is very time consuming in that it requires rather long immersion in successive acid baths with intermediate washing and scrubbing operations. Furthermore, pickling does not effectively clean the steels since it leaves their surfaces covered with smut, a black deposit which adheres tightly to the surfaces and must be removed by mechanical scrubbing. In addition to the lack of efficiency in cleaning the steels, the pickling method is also open to objection that spent pickling baths must be disposed of, a problem for which no entirely satisfactory solution has been found to date.

2

In view of the disadvantages of mechanical methods and acid pickling methods for the cleaning and descaling of such steels, attempts have been made and are still being made to utilize molten baths both with and without electrolysis for such purpose. The application of the cleaning methods involving electrolysis in fused baths to sheets has proved to be impracticable because of the large surface areas to be treated, the high current densities required, and the low voltage (6 to 8 volts) direct current that must be used. Attempts were next made by inventors to devise fused baths that would clean the steel effectively without electrolysis. Among such baths are the fused sodium hydroxide baths containing a minor proportion of a strong reducing agent, such as sodium cyanide or sodium hydride. Both of the last-named baths are hazardous to use, the first because sodium cyanide is a very poisonous substance and the second because the sodium hydride is formed in the fused bath by adding metallic sodium to a boxed-in section of the molten hydroxide bath and bubbling through the molten sodium hydrogen derived from the thermal decomposition of ammonia, which, if not complete, leaves ammonia which combines with the sodium to form the somewhat volatile sodamide. These baths, furthermore, are comparatively slow in action, requiring from 10 to 20 minutes' immersion to effect complete descaling of the class of steels mentioned above.

We have invented a novel fused bath useful in the removal of scale and oxides from such difficultly cleanable metals in the manner presently to be described, whereby not only are the hazards of the previously known baths avoided but the time of immersion required for descaling is materially reduced. By our invention, the average time of immersion is reduced to about three minutes. Our novel bath preferably has the following composition:

|                                                                         | Per cent by weight |
|-------------------------------------------------------------------------|--------------------|
| Alkali metal nitrate                                                    | 40 to 99.9         |
| Alkali metal nitrite                                                    | 0 to 60            |
| Alkali metal oxide (containing at least 2 atoms of oxygen per molecule) | 0.1 to 5.0         |

In the preferred embodiment the sodium salts and a higher oxide of sodium are employed because such materials are cheap and easily available. Specifically, it is preferred to use as the higher oxide sodium peroxide, so that at least

a predominant portion of the bath has the following composition:

|                                             | Per cent   |
|---------------------------------------------|------------|
| Sodium nitrate ( $\text{NaNO}_3$ )          | 40 to 99.9 |
| Sodium nitrite ( $\text{NaNO}_2$ )          | 0 to 60    |
| Sodium peroxide ( $\text{Na}_2\text{O}_2$ ) | 0.1 to 5.0 |

the percentages given being by weight.

While it is preferred that the bath consist at least substantially wholly, if not wholly, of the above composition, our invention also contemplates fused baths, and the use of such baths, in which there is also present, in minor amounts not affecting the action of the bath, other fused salts essentially neutral to the bath and the metal and oxide of the metal being cleaned.

All the compounds used in this bath may be of the ordinary commercial or technical grades, the only requirement being that the nitrate or nitrate-nitrite mixture used, preferably sodium nitrate, or a mixture of sodium nitrate and nitrite, must be dry and free of organic matter, and the alkali metal higher oxide, preferably sodium peroxide, relatively free of moisture, since either organic matter or moisture in or on any materials added to the bath will cause it to foam badly. The market prices of sodium nitrate and sodium nitrite are about the same as or slightly less than the market price of sodium hydroxide, and the cost per ton of sodium peroxide is generally near that of metallic sodium, so it is apparent that the bath of our invention can be operated to clean and descale steel at a cost per day no greater than the cost of operating the sodium hydroxide-sodium hydride bath. In addition, our bath requires no ammonia, operates at a lower temperature than the hydroxide baths, and cleans at a faster rate, so that the cost per ton of steel cleaned may be considerably reduced by the process of our invention.

Since the bath is extremely active, another requirement is that the pot or container in which the sodium nitrate is fused be made of materials that will resist chemical attack. The bath will cause a pot made of ordinary grades of carbon steel, as well as many high alloy steels, to fail within a few months to a year. Since the metals that show greatest resistance to the action of the bath are pure nickel, and the nickel alloys known as Monel metal and Inconel, a pot made of a low carbon steel clad with one of these metals on the inside is to be strongly recommended, especially since these metals are readily bonded to plain steel and the nickel or nickel alloy layer used not be more than one-twentieth of the thickness of the clad steel plate of which the pot is made. A pot made of such clad steel plates properly welded together and uniformly heated will last indefinitely.

The pot may be heated by any of the conventional methods in use, but the preferred method is by circulating hot gases, such as the products of combustion of a gaseous or liquid fuel, exteriorly about the walls of the vessel, through flues properly insulated to avoid loss of heat to the surrounding air. If the pot is heated electrically or with gas-fired radiant tubes, the heating elements must be made of materials to resist the action of the bath, preferably of nickel or of one of the nickel alloys mentioned. The pot may be of any dimensions desired and should be built to accommodate the largest size of article to be treated and leave sufficient space surrounding it so that the article may be completely immersed.

To start a bath of the preferred composition which is given only by way of example, the pot is thoroughly cleaned and dried, the requisite amount of sodium nitrate or the sodium nitrate-sodium nitrite mixture to be used is added and heat is applied gradually until the salt or mixture is melted and the fused bath has reached a temperature of 650° F., the minimum operating temperature. At this temperature sodium peroxide is added slowly and dissolves in the bath; at lower temperatures it remains unfused and settles to the bottom of the pot. The highest operating temperature is limited to about 800° F., because sodium nitrate starts to decompose at 716° F., but the decomposition progresses very slowly up to 800° F. A limiting temperature of 850° F. is no handicap, however, because the highest temperature to which steels of the stainless and corrosion and heat resistant types may be heated after the final heat treatment is 900° F. As a final treatment these steels, or such as contain more than 0.02% carbon, are heated to high temperature (1950° F. to 2200° F.) and quenched to hold carbides in solution, and subsequent heating to a temperature above 900° F. starts a precipitation of the carbides which reduces the corrosion resistance of the steel. Within the range 650° F. to 850° F., the activity of the bath and consumption of sodium peroxide increase as the temperature of the bath is raised, and above 800° F. the decomposition of the nitrate increases rapidly as the temperature is raised.

After the initial charge of the bath has been melted, more of the salt or salt mixture is added to fill the pot to a level that will permit complete immersion of the article or articles to be cleaned and descaled without raising the liquid level above a line 3 to 4 inches from the top. The temperature of the bath is then raised to the desired working temperature between 650° F. and 800° F., and a predetermined amount of sodium peroxide is added sufficient to give the concentration desired, usually 0.5% to 1.0% of the weight of the bath for batch type operation, unless it is desired to increase the activity of the bath, when peroxide equivalent to 3% of the weight of the bath may be added. High activity is desirable to reduce the time of immersion as when several lots of articles are to be cleaned in rapid succession, or when the scale to be removed is heavy or of a type difficult to remove. To save peroxide and thus reduce the cost, it is desirable to maintain the concentration of peroxide somewhat below 1% when the bath must stand idle for varying periods between treatments.

Assuming that the articles to be cleaned are stainless steel sheets, the operations to effect a complete cleaning and descaling of their surfaces are recited as follows: The sheets to be treated are set up edgewise upon a rack made of Monel metal or Inconel, and each sheet in the rack is prevented from making contact with the sheets adjacent to it, preferably, by means of grooves in the support bars of the rack and in a cross bar extending across the top. Alternatively, the sheets may be kept from contacting each other at the top by inserting short round separator bars between adjacent sheets. Since the effect of immersing cold sheets into the liquid bath is to cause the salts to solidify upon the cold surfaces, the rack of sheets is preferably preheated to the temperature of the bath to reduce the time of immersion required. The

racks used are of conventional design suspended from a cross bar or cross bars at the top which may be attached to the hook and chain of an overhead electric crane spanning the building in which all the treating equipment is housed. After the rack of sheets has been heated, it is transferred by the crane, lowered into the fused bath until the sheets are immersed, and the cross bar or bars rest upon the top of the pot. The sheets are permitted to remain in the bath, preferably to save time, no longer than necessary to dissolve the scale, although longer immersion does not harm the sheets, since the base metal of the latter is attacked but slightly by the bath. The exact time required to dissolve the scale varies from several seconds to three to four minutes, depending upon the temperature of the sheets when immersed, the thickness and character of the scale to be removed, the condition of the surface of the sheets, whether pitted or smooth, the type of steel being treated, the conditions of the previous heat treatment, and to a certain extent the temperature of the bath and the concentration of sodium peroxide. For example, to clean cold-rolled muffle-annealed sheets of 18-8 chromium-nickel steels immersed cold requires only two minutes, whereas three to four minutes are required to clean cold-rolled box-annealed sheets of straight 12 to 14% chromium steel immersed cold into the bath maintained at a temperature of 650° F. for both steels. For reasons to be explained later, concentrations of sodium peroxide varying from 0.1% to 1% have little effect upon the time required to clean either of these types of steel. As previously stated herein the time required to clean can be reduced somewhat by preheating the sheets to the temperature of the bath, and the removal of scale is also accelerated somewhat by moving the rack of sheets back and forth in the bath or by producing circulation of the bath between the sheets as with a submerged propeller. Therefore, some experience in operation of a bath and knowledge of the type of steel and the treatment it has received are necessary to permit an operator to determine in advance the exact time of immersion.

At the end of the immersion period the rack of sheets is raised out of and held over the bath for a short period to permit the molten salts to drain from them, when the rack of sheets is lowered into a water bath to cool them and remove soluble salts adhering to them. This treatment generally leaves the surfaces of the sheets coated with a thin red film of ferric hydroxide, which is removed by immersing the sheets in hot (140° F. or higher) dilute aqueous solution of sulphuric acid. As this treatment generally leaves the surfaces darkened with a smut, the rack of sheets is next dipped into a hot (120° F. or higher) dilute (2% or higher) aqueous solution of nitric acid, containing .05% or more of hydrofluoric acid. This treatment usually leaves the surfaces of the sheets with a bright metallic luster, the brightness and smoothness of which are largely determined by treatments prior to immersion in the cleaning bath. Following this treatment the sheets are rinsed by dipping them in clean water and if the surfaces are not uniformly bright, they may be passed through cloth polishing rolls. As a final step, the sheets may be dried to give a finish acceptable to the trade or adapted to any succeeding operation or processing.

To resume discussion of the fused bath, its

most efficient operation requires observance of certain precautions listed as follows:

Since the active chemical is sodium peroxide, it is necessary, for reasons to be explained later, to have a small excess of this reagent present in order to reduce the time of cleaning to a minimum, and since a large excess is not required and some is carried out of the bath with each lot of sheets treated, it is better to add this reagent in small lots just before immersion of each lot of sheets than to add a large quantity at the beginning of any one period of the day. Under such conditions, it is well to devise a quick chemical test for sodium peroxide, take samples from the bath at frequent intervals and make additions of peroxide as indicated by the results of these tests.

Raising the temperature of the bath above 650° F. increases its activity but also increases the consumption of sodium peroxide, particularly if and as the temperature is raised above 730° C., because the peroxide acts to oxidize or reoxidize sodium nitrite added to or formed in the bath. Since this action is relatively slow, adding the peroxide just before sheets are immersed in the bath helps to reduce the loss of peroxide from this cause.

The salts carried out of the bath with each lot of sheets treated is replaced at intervals by small additions of sodium nitrate. After a bath has been in use for a time the products formed by reactions of the peroxide or nitrate and peroxide with the scale are precipitated and settle to the bottom, so that it eventually becomes necessary to remove this sediment. This removal may be made in different ways, but a most convenient means consists of shallow rectangular pans made of nickel, Monel metal or Inconel, set in so as to completely cover the bottom of the pot and provided with large lugs along the sides so that they may be lifted by a crane from the bath as they become filled with sludge, emptied and replaced.

The treatments following immersion in the fused bath may be varied from those given above. For example, the red coating left upon the first immersion in water may be removed mechanically, by passing the sheets through a scrubbing machine. Also, after the fused salts have drained off, the sheets may be cooled in the air or with an air blast and then immersed into a bath of sulphuric acid to which a little hydrofluoric acid is added. In this treatment the sulphuric acid reacts with the sodium nitrate to form sodium sulphate and nitric acid and with any adhering sodium chromate formed in the fused bath to give sodium sulphate and chromic acid, and this single acid treatment followed by rinsing in boiling hot water may be all that is required to give the finish desired. In the treatment of sheets made from certain grades of steel by certain processes, such as 18-8 chromium-nickel steels muffle annealed, the dip in sulphuric acid may be omitted, and the red to reddish brown deposit left from the water wash may be removed by a single dip in a nitric or nitric hydrofluoric acid bath.

Regarding a choice between the straight sodium nitrate-base bath and the nitrate-nitrite-base bath, it would appear that the latter is desirable at the start only in special cases requiring a low temperature working range between 650° F. and 700° F. for the following reasons:

The melting point of sodium nitrate is given

75 at 584° F. and that of sodium nitrite as 572° F.

but a mixture of the two melts at a lower temperature than either alone, a fused mixture made of equal parts of sodium nitrate and sodium nitrite forming an eutectic that melts at about 432° F. Other mixtures containing from 30% to 50% sodium nitrate with the balance of sodium nitrite melts at temperatures between 440° F. and 450° F. With any of these mixtures heated to the minimum operating temperature of 650° F., the consumption of sodium peroxide appears to be somewhat less than in the straight sodium-nitrate base bath operating at the same temperature, but the chemical activity of the former bath appears to be slightly greater than that of the latter for the same concentration of sodium peroxide. Aside from these advantages, there is seldom any reason for starting with the nitrate-nitrite bath, because the first cost of the nitrite is usually three to four times that of the nitrate, and as will be shown later, the straight nitrate bath may be operated to form nitrite if desired.

From the foregoing description of the invention, it is obvious that it may be applied to the cleaning and descaling of numerous articles besides sheets, made of other ferrous metals as well as of the high chromium steels cited as examples of steels most difficult to descale. Furthermore, various modifications may be made in both the bath and the method without exceeding the scope of the invention. Thus, instead of sodium nitrate or a mixture of sodium nitrate and nitrite, the sodium salt or salts being preferred, as explained, because of their low cost, a nitrate or a mixture of a nitrate and a nitrite of the other alkali metals, potassium, lithium, rubidium, and cesium may be substituted in whole or in part and used in conjunction with either sodium peroxide or one of the higher oxides of the other alkali metals, of which the oxides of potassium represented by the formulas  $K_2O_2$ ,  $K_2O_3$ , and  $K_2O_4$  are representative. The particular alkali metal nitrate or nitrates, mixture of nitrate and nitrite or mixture of nitrates and nitrites, and higher oxide or oxides of an alkali metal chosen for the bath depend upon the melting point of the bath desired and the stability required of the bath. Ordinarily, to obtain baths which have melting points well below 900° F. and which are quite stable, it is preferred to employ the sodium nitrate or mixture of sodium nitrate and nitrite and sodium higher oxide, the corresponding potassium compounds, or mixtures of such sodium and potassium compounds.

It is possible to substitute other strong oxidizing agents, such as potassium or sodium chlorate or perchlorate, or potassium or sodium permanganate, for the higher oxide or oxides of the alkali metals in the fused bath of the invention. The use of such other oxidizing agents is ordinarily to be avoided, however, since in all instances their cost is greater than that of either the sodium or potassium higher oxides such as the peroxide. The action of such other oxidizing agents is in most instances such as to form a substance insoluble in the bath, thus adding to the amount of sludge formed. Many of such other oxidizing agents are poisonous, or at least are hazardous to handle. In the case of the chlorates and perchlorates, the introduction of chlorine into the bath by them causes foaming of the bath, which, of course, is undesirable. As a more serious disadvantage, the chlorine has a deleterious effect upon the steel to be cleaned and the container. In all instances the higher oxides of the alkali metals have been found to form a fused bath,

with the other recited components, which is not exceeded even initially in cleaning action by baths in which such other oxidizing agents, that is, the chlorates, perchlorates, and permanganates have been substituted for such higher oxides of the alkali metals. In addition, the bath of the invention is stable, free from hazard in the handling of the ingredients, and cheap.

Although it is to be understood that the method of cleaning and descaling ferrous articles and the bath therefore of the present invention are not to be defined, restricted, or confined to theoretical discussion, the following theory of operation which is supported by experimental evidence, is given as a means of distinguishing the present invention from others closely related to it and of aiding inexperienced operators to a better understanding of the process.

To understand the action of the bath, it is necessary to know the nature and composition of the scale to be removed. The scales formed on the surfaces of steels of the class and type under consideration from exposure to the usual heating furnace atmospheres are complex in character and vary in composition from the outer surface of the scale to the surface of the metal beneath. At the outer surfaces of scales thus formed on the steels of the straight chromium types are found intermingled the oxides of iron and chromium,  $FeO$ ,  $Fe_3O_4$ , and  $Cr_2O_3$ , with the probability that some of the  $FeO$  is combined with some of the  $Cr_2O_3$  as chromite,  $FeO \cdot Cr_2O_3$ , and with  $SiO_2$  as iron silicate, if the steel contains much silicon. In any case, the oxide of chromium,  $Cr_2O_3$ , makes up a major portion of this outer surface layer of scale. On steels of the chromium-nickel types, nickel oxide,  $NiO$ , will also be found in this outer surface layer intermingled with the other oxides. Beneath the outer surface layer the oxides exist mainly as  $FeO$  and  $Cr_2O_3$ , and if the steel contains nickel it is present as the metal, not the oxide, while the scale adjacent to the metallic surface consists of the lower oxides of iron,  $FeO$ , and chromium,  $CrO$ , intermingled with metallic iron, or metallic iron and metallic nickel, bonding the scale tightly to the metal.

As the chromic oxide in the outer surface layer of scale is insoluble in acids, it is very difficult to remove these scales by pickling, and since all the oxides in the scale are bases, they will not react with the alkali hydroxides or other bases in whatever manner these reagents may be applied.

In the fused baths of our invention, however, these scales and any carbonaceous or organic matter present are rapidly attacked, because the baths, whether of the nitrate-base or the nitrate-nitrite-base type, are intensely oxidizing and weakly basic in action. Fused baths of either sodium nitrate alone or any mixture of sodium nitrate and sodium nitrite in which the former is a major constituent are capable of strong oxidizing action, and the addition of sodium peroxide intensifies this action and, at the same time, makes the bath basic. How the action of the two is controlled in the practice of the present invention to remove the scale without appreciable attack upon the base metal of the article being descaled is explained as follows:

As previously explained, the scale as a whole on all types of the corrosion and heat resistant steels may be looked upon as an intimate mixture of the oxides of iron, chromium, and nickel with minute bodies of metallic iron and metallic

nickel intermingled with the oxides, the outer surface of the scale consisting of the oxides only. These oxides consist of the one oxide of nickel,  $\text{NiO}$ , two oxides of iron  $\text{FeO}$  and  $\text{Fe}_2\text{O}_4$ , and one oxide of chromium,  $\text{Cr}_2\text{O}_3$ . Toward all these oxides sodium nitrate is neutral, and sodium nitrate is neutral to all except the oxides of iron, which it oxidizes to ferric oxide,  $\text{Fe}_2\text{O}_3$ , thus:



Toward the metals, the nitrite may act as an oxidizing agent except chromium, but the nitrate effects surface oxidation of all by reactions represented as follows:



Sodium peroxide, however, is capable of oxidizing not only the metals and oxides to the same stage as sodium nitrate, but also of oxidizing chromium oxide to chromic anhydride, with which it or the sodium oxide formed in the reaction combines to form sodium chromate or sodium dichromate, as represented by the following reactions:



The excess sodium oxide formed in reaction 5, or other reactions of sodium peroxide, combines with ferric oxide to form sodium ferrite, thus:



Considering the reactions that may take place when sodium peroxide is added to the nitrate or nitrate-nitrite bath, we find that sodium peroxide may react alone to oxidize the chromic oxide and form either sodium chromate or sodium dichromate and sodium oxide, or react in combination with sodium nitrate to oxidize the chromic oxide and form sodium chromate and sodium nitrite; and that sodium oxide may react in combination with sodium nitrate to form sodium dichromate and sodium nitrite, which reactions are represented as follows:



Also, sodium peroxide may react directly with ferrous oxide to form sodium ferrite, thus:



and in the bath described herein it oxidizes sodium nitrite slowly, thus:



A thermodynamical study of these reactions indicates that reactions 9 and 11 are most likely to occur and a mere inspection of all shows that (a) only reactions 5, 9, and 10 give sodium oxide to combine with ferric oxide or chromic oxides, as in reactions 7, 8, and 12; (b) to accomplish the descaling by reactions 5, 6, 9, 10 and 13 requires that the bath contain at the time of immersing the steel an amount of sodium peroxide sufficient to react with the scale, probably a large excess, if means of circulating the fused salts are lacking; and (c) the bath is more or less self-adjusting in that, in the absence of sufficient so-

dium peroxide to react with all the scale, as in reactions 9 and 10, the sodium nitrate making up a major portion of the bath at all times may become active to assist in the descaling action in accordance with reaction 11; and if too great an excess of sodium peroxide is added, it may be consumed as in reaction 14, to restore the nitrate-nitrite balance of the bath. In making the sodium peroxide additions, therefore, the operator may aim at maintaining the minimum excess of peroxide required to effect the descaling in accordance with reactions 9 and 13, without fear of failure due to insufficient peroxide to react with all of the scale.

In these respects either the straight nitrate or nitrate-nitrite bath of the present invention differs from all others, and also holds an advantage in that, due to its chemical activity, it effects descaling in a much shorter time than any other bath. It also has an advantage over certain baths known heretofore in that it can be operated in safety and without hazard to the workmen. Neither the reagents nor the products of the reactions are classed as poisons, and the only special precautions it is necessary to observe in operating the bath is to protect the hands from contact with the sodium peroxide and avoid introducing water, carbonaceous or organic matter into the bath, any of which will cause it to foam.

A special advantage in operating the bath with a minimum of sodium peroxide is that the metallic surface beneath the scale is attacked but slightly. The sodium nitrate or nitrate-nitrite-base bath not only serves as a diluent of the peroxide, but also reacts with the surface metal, as represented by reactions 2, 3, and 4, to form a coating on the surface that acts to break contact of the liquid bath with the metal.

Among other advantages of the bath of our invention is the low temperature at which it may be operated and the fact that all the chemicals carried out of the bath on the surfaces treated, except the oxides of iron and nickel, dissolve rapidly in water to form a harmless solution that may be discharged into most streams with beneficial rather than deleterious effects upon either animal or vegetable life. An appreciable portion of the sodium chromate and ferrite formed dissolves in the bath where they accumulate until the bath becomes saturated with them, when they are precipitated. The drag-out and additions, however, tend to prevent such a build-up, with the result that sludge accumulates slowly.

The sodium ferrite carried out of the bath on the surfaces of articles treated reacts with water to form sodium hydroxide and ferric oxide, in accordance with the following reaction:



The ferric oxide remains on the surface with the nickel oxide and may be removed in part with high pressure water sprays, or in whole by scrubbing or by dipping in hot dilute sulphuric acid followed, if necessary, by a dip in hot dilute nitric hydrofluoric acid, as hereinbefore explained.

Having thus fully disclosed and described the cleaning and descaling method and bath therefore of our invention, we claim as new the following:

We claim:

1. The process of cleaning ferrous articles which comprises contacting the articles with a fused mixture relatively free of moisture and

organic matter, consisting essentially of the following composition given in percentages by weight:

|                                                                         | Per cent   |
|-------------------------------------------------------------------------|------------|
| Alkali metal nitrate                                                    | 40 to 99.9 |
| Alkali metal nitrite                                                    | 0 to 60    |
| Alkali metal oxide (containing at least 2 atoms of oxygen per molecule) | 0.1 to 5.0 |

2. The process of cleaning ferrous metals which comprises contacting the metal with a fused mixture relatively free of moisture and organic matter, consisting essentially of the following composition given in percentages by weight:

|                                                                         | Per cent   |
|-------------------------------------------------------------------------|------------|
| Alkali metal nitrate                                                    | 40 to 99.9 |
| Alkali metal oxide (containing at least 2 atoms of oxygen per molecule) | 0.1 to 5.0 |

3. The process defined by claim 2 characterized by maintaining said bath at a temperature between 650 and 800° F.

4. The process defined by claim 2 characterized by withdrawing the article from the fused bath and washing its surfaces with water; contacting the washed surfaces with dilute acids to remove any coating remaining thereon; exposing the surfaces to water to remove the acid, and finally drying the article.

5. The process defined by claim 1 characterized by withdrawing the articles from the fused bath, washing their surfaces to remove the coating

adhering thereto; and finally scrubbing the surfaces with water and drying the articles.

6. A cleaning bath for an oxide-coated ferrous metal article which consists essentially of a fused mixture relatively free of moisture and organic matter, having substantially the following composition in percentages by weight:

|                                                                         | Per cent   |
|-------------------------------------------------------------------------|------------|
| Alkali metal nitrate                                                    | 40 to 99.9 |
| Alkali metal nitrite                                                    | 0 to 60    |
| Alkali metal oxide (containing at least 2 atoms of oxygen per molecule) | 0.1 to 5.0 |

MATTI H. PAKKALA.  
FREEMAN J. PHILLIPS.

15

References Cited in the file of this patent

UNITED STATES PATENTS

| Number    | Name         | Date          |
|-----------|--------------|---------------|
| 1,714,879 | Lang         | May 28, 1929  |
| 2,244,526 | MacKay       | June 3, 1941  |
| 2,311,099 | Tainton      | Feb. 16, 1943 |
| 2,395,694 | Spence       | Feb. 26, 1946 |
| 2,538,702 | Noble et al. | Jan. 16, 1951 |

25

FOREIGN PATENTS

| Number  | Country       | Date         |
|---------|---------------|--------------|
| 466,661 | Great Britain | May 26, 1937 |

30

OTHER REFERENCES

Condensed Chemical Dictionary — Reinhold Pub. Co., N. Y., 3rd Edition (1942) p. 588 (Copy in Scientific Library).